

Aug. 11, 1931.

L. T. WORK ET AL

1,818,184

ELECTRICAL RESISTANCE COMPOSITION

Filed June 14, 1929

252-490



Fig. 1.



Fig. 2.



Fig. 3.



Fig. 4.

Fig. 5.



Fig. 6.

INVENTORS,  
 Lincoln T. Work  
 Elmer S. Imes  
 BY Edgar A. Everett  
 M. A. Longfellow  
 ATTORNEY

X R.

## UNITED STATES PATENT OFFICE

LINCOLN T. WORK, OF YONKERS, ELMER S. IMES, OF NEW YORK, AND EDWARD A. EVERETT, OF LONG ISLAND CITY, NEW YORK; SAID WORK AND SAID IMES AS SIGNORS TO SAID EVERETT

## ELECTRICAL RESISTANCE COMPOSITION

Application filed June 14, 1929. Serial No. 371,044.

This invention relates to an electrical resistant material formed from a composition in blocks and shapes and with varying characteristics. This material may be made to have a comparatively high resistance, or it may be varied in its composition to have a comparatively low resistance so that it may be used as a substitute for resistance coils, or for carbon resistance units, for general purposes in an electric circuit.

10 This composition is usable as a resistance unit in electric circuits of varying capacities according to the content of the composition and to the cross-section used as a conductor. As the material may be drilled, ground and machined, its cross-section can easily be regulated with considerable precision. It may also be mounted in separate units of varying sizes for different capacities.

20 This composition as produced in blocks is practically impervious to moisture, that is; it will absorb only a low moisture content. However, in practice it may be saturated to this extent with a conducting salt, preferably 25 silver nitrate, ( $AgNO_3$ ), by steeping in a suitable solution, and, as this material is not stable under the action of light, it may be stabilized by subjecting the blocks, after steeping, to the fumes of hydrogen bisulphide ( $H_2S$ ), changing the impregnation to silver sulphide ( $Ag_2S$ ). Under the microscope it is found that this impregnation saturates the whole content and increases the conductivity uniformly, which is desirable 35 for the purpose intended.

The construction and application of this invention will be more fully understood from a consideration of the following specification and the accompanying drawings, selected to illustrate a form of the invention applied to resistance units, and in which,

40 Figs. 1, 2 and 3 illustrate various forms that this invention may take as applied in use.

45 Figs. 4 and 5 show this invention applied to a form of adjustable non-inductive resistance and

Fig. 6 is a form of fixed resistance with electrical connections at intervals.

50 This invention is concerned mainly with the manufacture of the resistance block. The

blocks are composed of a binder and a conducting medium mixed together in finely divided form in the proportions desired. When the binder is set, the blocks are moulded under pressure and afterwards "cured". Heat is not used in the process, except in the curing as hereinafter specified.

55 The binder is composed of Portland cement, finely ground. Cement has given satisfactory results for this purpose. Various materials may be used for the resistance aggregate according to the characteristics desired in the final product. The following materials are recommended for this purpose: Mineral black, powdered graphite and powdered carborundum.

60 Mineral black which is a carbonaceous shale is found to have a decided decrease in resistance with increase in temperature. Graphite has a better conductivity than mineral black and is preferred for low resistance blocks, but it is somewhat more difficult to mix with the binder.

70 The following proportions give a block having the characteristics of resistance, strength and durability desired:

75 50 grams Portland cement, 10 grams mineral black,  $16\frac{1}{2}$  c. c. water.

80 The two powders are mixed first and the water is then incorporated with it. The wet powder is compressed into the mould at the pressure ranging between 2,500 and 25,000 lbs. per square inch. The amount of water needed may vary slightly with the pressure used. The mixture is known as the "dry process" i. e., it does not flow as a liquid and is therefore easy to handle in the mould.

85 After removing from the mould, the blocks are "seasoned" by supplying additional moisture. This preferably is done by the application of a jet of steam for about five hours which penetrates the blocks and insures a thorough setting of the cement. Without this seasoning the blocks are inclined to crumble, are more fragile and their mechanical resistance is lowered. However the addition of asbestos fibre to the mix reduces the brittleness. The blocks are placed in a wire basket and enclosed in the steam chamber during the seasoning process. The blocks

55

60

65

70

75

85

90

95

100

may be air dried for a few days after the seasoning process or they may be further cured under water for a time and used after drying out.

Blocks of this composition have been subjected to certain tests to determine their characteristics, as given in the table below. The air dried blocks were used as taken from the mould, after drying in the air and without seasoning. These blocks do not have the desired mechanical strength. The moist dried-water cured blocks were dried in air as they came from the mould and afterwards steeped for three or four days in water and then dried out before testing. The steam dried-water cured blocks were subject to a jet of steam as described and then immersed in water for a few days. It has been found that in the latter treatment the water immersion makes very little impression on the block, in fact, the extent to which the blocks absorb moisture is governed by the pressure used on the mould. The composition is close in the grain and under high pressure the moisture absorption is very low.

The characteristics of this composition will be understood from the following tests:

| 30 | Composition                                     | Treatment                     | Resistance<br>in ohms<br>dry |
|----|-------------------------------------------------|-------------------------------|------------------------------|
|    | (a) 83.3% Portland cement, 16.7% mineral black. | Air dried.....                | 12,000                       |
|    | (b) Same as (a).....                            | Moist dried, water cured..... | 30,000                       |
|    | (c) Same as (a).....                            | Steam dried, water cured..... | 100,000                      |
|    | (d) 83.3% Portland cement, 16.7% lampblack      | Air dried.....                | 2,000                        |
| 35 | (e) Same as (d).....                            | Moist dried, water cured..... | 5,000                        |
|    | (f) Same as (d).....                            | Steam dried, water cured..... | 8,000                        |
|    | (g) 83.3% Portland cement, 16.7% wood charcoal. | Air dried.....                | Infinity.                    |
|    | (h) Same as (g).....                            | Moist dried, water cured..... | 150,000                      |
|    | (i) Same as (g).....                            | Steam dried, water cured..... | 20,000,000                   |
|    | (j) 83.3% Portland cement, 16.7% graphite.      | Air dried.....                | 25,                          |
| 40 | (k) Same as (j).....                            | Moist dried, water cured..... | 270,                         |
|    | (l) Same as (j).....                            | Steam dried, water cured..... | 150,                         |
|    | (m) 71.4% Portland cement, 28.6% corborundum.   | Air dried.....                | 11,000,000                   |
|    | (n) Same as (m).....                            | Moist dried, water cured..... | 1,400,000<br>to 800,000      |
|    | (o) Same as (m).....                            | Steam dried, water cured..... | 600,000<br>to 900,000        |
| 45 | (p) 83.3% Portland cement, 16.7% corborundum.   | Air dried.....                | 8,000,000                    |
|    | (q) Same as (p).....                            | Moist dried, water cured..... | 150,000                      |
|    | (r) 95% Portland cement, 5% lampblack.          | Moist dried, water cured..... | 8,000,000                    |
|    | (s) Same as (r).....                            | Steam dried, water cured..... | 9,000,000                    |

50 In general, it will be noted from the above tests that the electrical resistance of the material depends upon the composition, and upon the process of manufacture. The lower the content of the conducting material the higher the resistance; also, air dried blocks are usually lower in resistance than moist dried or steam dried; and moist dried and water cured blocks are usually lower in resistance than steam dried, water cured blocks.

55 Thus the electrical characteristics of the material can be varied either in the mix, or in the process of treating after the blocks are moulded. This enables resistance blocks to be made for a great variety of purposes and

60 in a variety of shapes.

Some of the common shapes of these blocks, for general use, are illustrated at 15, 16 and 17, Figs. 1, 2 and 3.

A common form of non-inductive resistance is shown in Figs. 4 and 5 in which the present compound, preferably using lampblack or graphite as the conducting element is used in the ring shaped band 19 mounted on the insulated base 18 and connecting with the terminal 22. The knob 23 is centrally mounted in this ring and carries the contact arm 24 in engagement with 19, also the contact arm 25 in engagement with the metallic ring 20 which connects to terminal 21. The arms 24 and 25 are electrically connected through the stem of the knob 23. It is apparent that the resistance of the circuit between terminals 21 and 22 is varied by the movement of knob 23 to vary the portion of the resistance 19 that is included in the circuit.

A form of non-adjustable but variable resistance is shown in Fig. 6 in which the central bolt 74, through the insulated bushings 75 and 76 holds the parts together in cylindrical form. These parts comprise tubular sections 69, 70, 71 and 72 of various lengths of resistant material. These sections are mounted on the metallic collars 62, 63, 64, 65 and 66 and each of these collars are connected with a terminal as indicated at 67 and 68. Conductors may be connected to these terminals to include various lengths of resistant material in the circuit as desired.

55 It will be understood that this product is capable of being moulded and is capable of being machined so that it can be produced in almost any desired shape to very close limits. This, together with the fact that a homogeneous mix is readily obtained, enables resistance of precision to be produced by this invention.

The function of the Portland cement is to provide a binder having the required mechanical strength for the resistant material which is applied to the composition in powder form. Other binders may be used for this purpose such as "dental cement" which has great mechanical strength, or gypsum which is comparatively soft and easily moulded.

Having thus described our invention, we claim:

1. An electrical resistance material comprising a mixture of 50 grams Portland cement, 10 grams mineral black and 16½ c. c. water which has been moulded under pressure and seasoned by the application of additional moisture.

2. An electrical resistant material comprising a mixture of Portland cement with powdered mineral black and water which has been moulded under pressure to the shape desired.

3. An electrical resistant material com-

prising a mixture of 50 grams Portland cement, 10 grams mineral black and water which has been moulded under pressure to form.

5 4. An electrical resistant material comprising a binder of Portland cement and a conductor of pulverized mineral black mixed together with asbestos fiber and water and which has been moulded to shape under pressure and cured, after moulding, by the application of additional moisture.

10 In testimony whereof we affix our signatures.

15 LINCOLN T. WORK.

ELMER S. IMES.

EDWARD A. EVERETT.

20

25

30

35

40

45

50

55

60